

Jan. 9, 1923.

O. FISCHER.

1,441,569.

COLLECTOR FOR DYNAMOS AND THE LIKE AND PROCESS FOR MAKING SUCH COLLECTORS.  
FILED AUG. 12, 1921.

*Fig.1.*



*Fig.2.*



INVENTOR  
OTTO FISCHER

BY ATTORNEYS

Locke, Kellentick & Mathe.

## UNITED STATES PATENT OFFICE.

OTTO FISCHER, OF STUTTGART, GERMANY, ASSIGNOR TO ROBERT BOSCH AKTIEN-  
GESELLSCHAFT, OF STUTTGART, GERMANY.

COLLECTOR FOR DYNAMOS AND THE LIKE AND PROCESS FOR MAKING SUCH  
COLLECTORS.

Application filed August 12, 1921. Serial No. 491,851.

To all whom it may concern:

Be it known that I, Otto Fischer, German subject, residing at Stuttgart, Germany, have invented certain new and useful Improvements in Collectors for Dynamos and the like and Processes for Making Such Collectors (for which patents have been applied for in Germany, application filed April 29, 1919; Holland, April 24, 1920; Sweden, June 10 14, 1920; Switzerland, June 12, 1920; Austria, June 14, 1920; Czecho-Slovakia, June 16, 1920; Italy, June 22, 1920; Great Britain, June 22, 1920; Belgium, July 2, 1920; France, July 9, 1920), of which the following is a 15 specification.

The invention relates to the manufacture of collectors (for dynamos, motors, etc.) with bushings consisting of an insulating substance such as porcelain, steatite, bakelite or 20 the like upon which the copper segments are formed by a galvanic precipitation process. The general idea of producing segments through galvanic deposits is known and the practical procedure hitherto consisted in 25 covering the collector bushing with a layer of enamel and in thereupon applying protochloride of gold to the surfaces that were to receive the conducting segments, this gold then being fixed by annealing. The surfaces 30 thus covered with protochloride of gold were then thickened in an electrolytic bath by galvanic deposits.

In comparison with this known collector producing process the new process according 35 to the invention is much simpler. It enables the collectors to be made quicker and cheaper and with segments with well defined borders, which was not possible with the old process.

A special coating of enamel is not necessary with the process according to the invention, and the segments need not be prepared for the subsequent electrolytic bath by applying a special covering of protochloride of gold for each individual segment.

An important feature of the invention consists in covering, by a galvanic or other process, the entire periphery of the body of the collector, which is made of a suitable insulating substance, with a coating of metal

and in forming the various segments by 50 cutting up the integral copper coating with a saw. The collector segments thus produced are separated by well defined gaps and the rough edges formed at the gaps by the saw afford a safeguard against lateral movements 55 of the segments. Further security against lateral movement may be provided in the shape of grooves formed upon the circumference of the collector bushing. The galvanic coating preferably extends so 60 far over the collector bushing that it embraces the bushing at the ends and is thus safeguarded against the action of the centrifugal force set up when the collector rotates. If the collector bushing is made of 65 bakelite or any other substance that can be worked by tools, the segments can be produced without any further measures by cutting up the integral copper coating with a saw. But if (to obtain a great resistivity to 70 heat) steatite or some other ceramic substance is employed, grooves are formed in the substance previous to the baking of the same and while it is still soft, in order to render 75 it possible to cut up the subsequently deposited copper coating without the saw being damaged by the hard baked steatite substance.

In the drawing a constructional form of collector made in accordance with the invention is shown.

Fig. 1 representing a longitudinal section, and

Fig. 2 an end view of the collector or commutator.

The material used for the collector body or bushing is either a kind of insulating substance such as bakelite that can be worked by tools or, if it is to be capable of resisting high temperatures, a ceramic substance, such 90 as steatite, porcelain or the like, is employed, which is shaped as required before baking, due allowance being made for shrinkage.

If bakelite is used for the core of the collector bushing, the latter is finished on a 95 lathe—with the exception the grooves *b* that are afterwards made with a saw—and the whole periphery and inwardly extending lat-

eral surfaces *d*, *e* of the bushing are then provided with a coherent coating of conducting graphite, after which the bushing is immersed in a galvanic bath in which a coating 5 of copper is deposited upon the graphited surface. The copper coating of the brush surface of the collector is preferably made thicker than the lateral gripping coatings, this being accomplished by applying a coating 10 of varnish or the like to the side surfaces (as soon as they have become thick enough to securely hold the segments in place) and by subsequently continuing the galvanic process until a sufficient thickness of the brush 15 surface of the collector is attained. To obtain a smooth surface the integral copper coating is then shaved in a lathe and then subdivided into the required number of segments by cutting deep grooves *b* with a saw. 20 In order to prevent copper or graphite particles from accumulating in the grooves these latter are filled with cement or some kind of special insulating substance capable of resisting heat. The shallow grooves *c* in the 25 lugs of the segments are also made with a saw or cutter, but only deep enough to allow the wires of the armature to be conveniently soldered to them.

But if the substance used for the collector bushing is steatite, porcelain or another 30 ceramic material, deep grooves *b* for separating the segments, and shallow grooves *c* for fixing the armature wires are formed in the bushing whilst it is still soft. The bushing 35 is then baked, due allowance being made for shrinkage. The deep grooves are then filled with ordinary putty so as to prevent the depositing of copper therein during the galvanizing process. It is not absolutely necessary 40 to fill the grooves *b* with cement or the like, but this is the preferred procedure because if this were not done it would afterwards be necessary to carefully remove with a file or the like any layer of copper that 45 might have been formed during the electrolytic process.

After an integral coating of copper has been deposited on the bushing, and when the 50 surface of this coating has been shaved smooth with a turning tool as described, the copper deposit is cut up at the grooves *b* and *c* with a saw, which also removes the filling substance from the grooves. By thus providing grooves in the steatite previous to 55 the baking process, the copper coating can be completely cut into segments with a saw or cutter without the tool being damaged by the hard steatite.

It is obvious that the new process may 60 also be used for producing current distributing disks, switch plates, etc. To make the collector fit exactly on the armature shaft its bore may be provided with a metal bushing. A sleeve of glazed cardboard may be 65 inserted between the metal and the steatite

bushings. To obtain copper segments that are very securely fixed on the ceramic bushing a covering of protocloride of gold which is fixed by annealing may be used instead of the coating of graphite. The coating 70 of copper might also be put on by the Schoop squiring process or in any other way without departing from the spirit of the invention, but the copper deposited by a galvanic process is specially adapted for collectors on account of its hardness. 75

The term "collectors" in the following 80 claims is intended to cover all similar contrivances used for commutating or distributing electric currents, etc.

I claim:

1. A process of producing collectors consisting in forming the body of the collector of a suitable insulating substance, in covering the surface of the body with an integral 85 metallic coating, and in subsequently forming metallic segments by cutting up the coating.

2. A process of producing collectors consisting in forming the body of the collector 90 of a suitable insulating bushing, in covering the periphery of the bushing with an integral metallic coating, and in subsequently forming metallic segments by cutting up the coating with a saw.

3. A process of producing collectors consisting in forming the body of the collector of a bushing of soft ceramic substance, dividing the periphery of the soft bushing 100 into segments by making grooves in the periphery, hardening the soft bushing by baking it, covering the entire periphery with an integral metallic coating, and in finally cutting up the integral metallic coating at the said grooves so as to form metallic segments. 105

4. A process of producing collectors consisting in forming the body of the collector of a bushing of soft ceramic substance, dividing the periphery of the soft bushing 110 into segments by making grooves in the periphery, hardening the soft bushing by baking it, filling the grooves with a plastic substance, covering the entire periphery with an integral metallic coating, and in finally sawing up the integral metallic coating 115 at the said grooves so as to form metallic segments and remove the plastic substance.

5. In a collector made by the process 120 claimed in claim 1, inwardly-projecting lateral surfaces at the ends of the bushing, and inwardly-projecting extensions of the metallic segments engaging with the said inwardly-projecting lateral surfaces, whereby 125 the segments are prevented from being dislodged by centrifugal force.

6. In a collector made by the process 130 claimed in claim 1, inwardly-projecting lateral surfaces at the ends of the bushing, in-

wardly-projecting extensions of the metallic segments engaging with the said inwardly-projecting lateral surfaces, a peripheral groove in the said bushing, and an inward 5 bulge in each segment engaging with the said groove, whereby the segments are prevented from being dislodged.

In testimony whereof I have affixed my signature in presence of two witnesses.

OTTO FISCHER.

Witnesses:

ALFRED MEYER,  
HELMA PANDER.